

W. McA. JOHNSON.  
METALLURGICAL PROCESS.  
APPLICATION FILED SEPT. 20, 1909.

1,107,310.

Patented Aug. 18, 1914  
2 SHEETS—SHEET 1.



FIG. 1

WITNESSES:

Wm. M. Johnson  
Paul A. Woff

INVENTOR  
W. M. Johnson  
B  
DANIEL G. FISHER & SONS  
ATTORNEYS

W. McA. JOHNSON.  
METALLURGICAL PROCESS.  
APPLICATION FILED SEPT. 20, 1909.

1,107,310.

Patented Aug. 18, 1914

2 SHEETS-SHEET 2.



FIG. 2.

WITNESSES:

Norman D. Price  
Paul A. Clegg

INVENTOR

W. McA. Johnson  
BY  
Daniel C. Field & Son  
ATTORNEYS.

# UNITED STATES PATENT OFFICE.

WOOLSEY McA. JOHNSON, OF HARTFORD, CONNECTICUT.

## METALLURGICAL PROCESS.

1,107,310.

Specification of Letters Patent. / Patented Aug. 18, 1914.

Application filed September 20, 1909. Serial No. 518,530.

To all whom it may concern:

Be it known that I, WOOLSEY McA. JOHNSON, a citizen of the United States, residing at Hartford, in the county of Hartford and State of Connecticut, have invented 5 certain new and useful Improvements in Metallurgical Processes, of which the following is a full, clear, and exact description, such as will enable others skilled in the art 10 to which it appertains to make and use the same.

This invention deals broadly with a metallurgical process whereby an ore rich in a metalloid such as arsenic as well as either 15 nickel or cobalt and perhaps other valuable constituents may be commercially treated so as to enable its various constituents to be readily separated and otherwise refined. Inasmuch, however, as many of the noteworthy 20 advantages characteristic of this invention prominently appear in its more intense aspect as a metallurgical process especially applicable to the treatment of the extremely valuable and yet very intractable ores of 25 the Temiskaming region, some of which contain around about 35% arsenic, 10% cobalt, 5% nickel, 10% silver and a valueless residue containing silica and some carbonates, as of calcium, it will be conducive to clearness 30 to disclose the invention by way of a detailed discussion of such an embodiment thereof.

The invention accordingly consists in the features of construction, combinations of 35 elements and arrangement of parts which will be exemplified in the construction hereinafter set forth, and the scope of the application of which will be indicated in the following claims.

40 In order that this invention may be more readily disclosed and rendered comprehensible to those skilled in this art, drawings exemplifying two forms of apparatus suitable for acting as a means instrumental in carrying out this process are shown, and in 45 such drawings:

Figure 1 shows a horizontal furnace or retort for the chloridizing operation, in which the ore is reacted upon while in a 50 quiescent state; Fig. 2 is a form of tower which may be employed for the chloridizing operation and in which the ore, while rapidly falling through the tower in the form of a shower and while thus in a state of 55 movement is nevertheless in a condition

capable of precluding granular agglomeration at the temperature specified.

In case the ore should contain carbonates such as those of calcium and magnesium in such amounts as may be preliminarily advantageously reduced or eliminated, it is preferable to first subject the ore to the action of some such agent as hydrochloric acid in aqueous solution so that the contained lime may be brought into solution 60 and thus separated out, leaving an undissolved residue which may then be subjected to the following step of my process, or mechanical concentration on Wilfley tables may be employed.

In order to adequately comprehend the commercial importance of the next step of my process, it may here be noted that it is of the utmost consequence that the various steps or stages of any process, particularly 70 when formulated for the purpose of commercially refining ores displaying the perplexing metallurgical obstinacy characteristic of ores of the Temiskaming region, shall be selected or devised with a more 75 especial regard to the relationship or co-action therebetween. That is to say, it is imperative that an early step or sub-stage of the process must not only be adapted to adequately meet the immediate exigency but 80 must, furthermore, leave or bring the material or residue to be subsequently treated in such physical and chemical condition that the succeeding steps of the process may be 85 not only readily carried out but, also, that 90 such steps *per se* may be comparatively simple and essentially practicable from a chemical or metallurgical standpoint. Take, for example, an ore such as that under 95 present consideration, it is perhaps possible to devise a process which will serve to efficiently extract silver contents by means of certain individual steps which may be comparatively simple and yet such a process may have the very serious objection of leaving residues containing, say, nickel and cobalt in such physical and chemical form as to render the complete separation or purification of these valuable ingredients extremely difficult if not commercially impracticable.

100 It is, therefore, a primary object of this invention to so devise and relate the various steps of my process as to maintain or procure not only simplicity and effectiveness in 110

the steps *per se*, but, also, a commercially efficient and metallurgically harmonious relationship between such steps so that they will all co-act to the best advantage.

5 This invention, therefore, proposes as an early step of my process, the utilization of a gaseous chloridizing agent, such, for instance, as moist chlorin gas. In carrying out this stage of my process, the ore or residue containing high percentages of arsenic, silver, nickel and cobalt will be first obtained in a granulated or comminuted condition and then, while at a temperature varying from 250° C. to 350° C. and in what 10 15 20 25 30 35 40 45 50 55 60 65 70 75 80 85 90 95 100 105 110 115 120 125

may be termed a precluding granular agglomeration state, subjected for a period of time varying from ninety minutes to three hours, to the action of moist chlorin gas in the presence of aqueous vapor. As a result of my extensive investigations, I have discovered that efficiency and acceleration of action is greatly promoted by maintaining the above mentioned conditions, *i. e.*, using wet chlorin gas in connection with ore handled in such manner as to prevent or avoid the violent collision of particles, which would tend to cause cohesion of the granules. By this term "granular non-agglomeration" as employed in my specification and claims, I, therefore, mean an ore either contained in a suitable vessel or on shelves in a quiescent state, as well as ore in such a state of movement such as that obtained by permitting the ore to fall through a tower such as that shown in the annexed drawings, which movement will not tend to repeatedly rub or roll the particles together and cause granular cohesion, as contradistinguished from the ordinary rotating or tumbling methods, or mechanically rabbed furnaces, so frequently employed in connection with metallurgical roasting.

I have ascertained that when an ore of the specific character herein mentioned is subjected to the action of chlorin gas at a temperature of about 350° C. and upward, that the surfaces of the particles of such ore are in a more or less pasty condition and the effect of tumbling or rolling such ore is to 45 50 55 60 65 70 75 80 85 90 95 100 105 110 115 120 125

cause the various particles thereof to cohere and agglomerate to such an extent as to not only interfere with the complete chloridization of the ore and the volatilization of the arsenic but, also, to cause such ore to cling to the sides of the roasting vessel and be otherwise brought into a condition unadapted for subsequent handling and treatment.

In chloridizing the ore or residue it is 60 65 70 75 80 85 90 95 100 105 110 115 120 125

preferable to pass the chlorin gas through a tube having its end terminating below the surface of a body of water contained in a transparent receptacle, so that the chlorin may not only be suitably moistened but its flow readily observed by the rate at which

it bubbles up through the water. By observing the outlet from the roasting and chloridizing chambers the operator will be enabled to note whether or not excess of chlorin is passing through the apparatus. I have found, however, that the chlorin acts very completely and energetically on the ore, not only quickly chloridizing the directly exposed surface of the ore but extending into the interior portions thereof with great ease apparently by virtue of a sort of catalytic or carrier action. The reaction being exothermic in nature, the temperature tends to rise rapidly beyond that which my discoveries have set as proper limits below which a consequential amount of silver chlorid may volatilize and an undesirable agglomeration of the ore may take place, and I therefore have adopted the herein described step and means for maintaining the proper working temperature, which is about 350° C.

An embodiment of an apparatus suitable as a means instrumental in subjecting the ore to the action of moist chlorin gas at a carefully controlled predetermined temperature is diagrammatically illustrated by Fig. 1. Such apparatus consists of a furnace A containing a plurality of retorts B. This furnace A may be constructed of suitable heat resisting material, such as fire-brick or the like, and may provide a retort chamber 1 formed by the side walls 2, the arch 3, and the floor 4. The arch 3 and the floor 4 will preferably provide a number of vents or flues 5 and 6, respectively, to enable the temperature controlling air or gases to be brought into intimate contact with the walls of the retorts. To this end, the furnace A will preferably provide a wall 7 arranged to leave a space 8, which serves as a conduit for the entering, heat controlling air, and in like manner a wall 9 is arranged to form a conduit 10 for the discharge of the heat controlling gases. The retorts B may be suitably shaped, as for instance in the form of an ordinary muffle, and will each contain one or more perforated trays 11 supported on suitable blocks 12, or otherwise. These perforated trays are to be covered with ore, then placed in the retorts and the latter very carefully sealed up so as to prevent any escape of the poisonous arsenic chlorid. At 13 is shown a pipe serving as a conduit for admitting the moist chlorin gas to the first retort. This retort is connected with the next one of the series by means of a conduit 14 of fire-clay or the like, and in like manner the successive retorts of the series are connected together, the last one being connected with the pipe 15 through which the gaseous arsenic chlorid is withdrawn from the system. In this connection it should be observed that the entire system is preferably arranged to work under a slight negative 130

pressure by using suction-pumps or the like for withdrawing the arsenic chlorid, so that no arsenic chlorid may escape through crevices or the like in the roasting furnace 5 and possibly produce injury to the workmen.

Fig. 2 illustrates an embodiment of an apparatus also designed to serve as a means instrumental in efficiently chloridizing the ore. Such apparatus consists of a tower C 10 constructed of suitable heat resisting material, as of fire-brick. The circular or otherwise contoured wall of said tower preferably contains one or more continuous passageways 20 arranged on the inner surface 15 of the wall and through which the heat controlling gases may be passed so as to keep the temperature within proper limits. At the top of this tower some suitable ore delivering apparatus is arranged, such as, for 20 example, a hopper 21 having a perforated bottom 22 (which may be of about 100 mesh) and mounted on springs 23 so as to be capable of agitation. A rotating cam 24 is suitably arranged to agitate the hopper 21. 25 Preferably, this hopper is so arranged as, by means of a plate 25, to maintain a closure of the opening and thus prevent the escape of arsenic chlorid. The ore sifted through the bottom of the hopper falls through the 30 central chimney-like way of the tower until it reaches the bottom 26, which is so constructed as to enable it to be withdrawn. This ore will be preferably of one hundred mesh, so as to enable the chlorin gas to have 35 a complete action. At the bottom of the tower there are provided one or more conduits 27 through which is admitted moist hot chlorin gas and, preferably, the ore itself is maintained at as high a temperature as 40 may be practical, so as to prevent any chilling effect and enable the reaction to be carried out immediately. The temperature at which the interior of the tower is to be maintained is approximately 350° C. It has 45 been ascertained by experiment that the ore in thus falling through a tower of a height of, say, fifteen or twenty feet, is completely chloridized and gaseous arsenic chlorid may be withdrawn from the upper part of the 50 tower through the conduit 28. The chlorin gas thus acting on the ore transforms its constituents to chlorids, leaving a porous, granulated like residue each particle of which is somewhat puffed out. The arsenic, 55 however, has been changed to arsenic-chlorid  $\text{AsCl}_3$ , which is a heavy, yellowish liquid having a specific gravity of 2.6 and which because of the fact that its boiling point is at atmospheric pressure (136° C.) will pass 60 off as a vapor. This vapor is, of course, exceedingly poisonous and, therefore, I have devised a precautionary apparatus adapted to receive and take care of this poisonous vapor. That is to say, this arsenic chlorid

is preferably passed into a chilling room 65 where it is subjected to the action of jet condensers, or surface condensers, and enabled to re-act with water so as to be transformed into the insoluble arsenious acid  $\text{As}_2\text{O}_3$ , which is filter pressed and removed 70 as a by-product. The reaction is assumed to be as follows:



The porous, granular residue is withdrawn 75 from the chloridizing tubing or chamber when the arsenic contained therein has been expelled in the manner above indicated and will now be found to be in a condition admirably adapted for further treatments aiming particularly toward the isolation in commercially desired forms of the remaining valuable constituents of such residue. For example, it will be found that such ingredients have been all transformed into chlorids 80 which, with the exception of the silver chlorids, are readily soluble in slightly acidulated water. Therefore, as the next step of my process, this porous, granular residue containing very high percentages 85 of silver, nickel and cobalt may be leached with water acidified with from  $\frac{1}{2}\%$  to 5% of hydrochloric acid. The valuable ingredients, with the exception of the silver, which is in the form of the insoluble silver chlorid, 90 will immediately pass into solution, leaving a residue of silver chlorid mixed with more or less silicious matter from which it is, of course, readily separable. The solution may contain some slight traces of arsenious acid 95 100 which will preferably be precipitated by passing hydrogen sulfid gas into such solution and filtering off the precipitate as by means of a sand filter. The resultant solution will contain ferrous chlorid  $\text{FeCl}_2$ , nickel chlorid  $\text{NiCl}_2$ , and cobalt chlorid. The iron may very conveniently and efficiently be separated out by first transforming the same from the ferrous to the ferric condition by introducing enough chlorin gas 105 into the solution to oxidize the iron to  $\text{FeCl}_3$  and then milk of lime may be added and the solution agitated so as to precipitate the iron in the form of ferric hydrate  $\text{Fe}_2(\text{OH})_6$ . The filterate from the above 110 mentioned iron hydrate will now contain all of the nickel and cobalt and these two substances may be separated by known methods, as oxychlorid of lime or by chlorin gas and soda ash.

The residue from the chloridizing operation, as has been observed, contains silver chlorid and is thus well adapted for subsequent treatment whereby the silver may be readily obtained therefrom. Thus, this 125 residue may be treated by subjecting the same to the action of potassium cyanid and electrolyzing, or the silver may be obtained

from the potassium silver cyanid solution by means of zinc or aluminum shavings in the usual manner.

Viewed in the light of current knowledge and without the necessity of further elaboration, the foregoing disclosure will be sufficiently suggestive and otherwise enable those skilled in the art to easily devise certain interchangeably available embodiments and utilizations of this invention which, although perhaps calculated to seem dissimilar, and possibly performed by means of apparatus differing considerably in detail and appearance from that herein shown, would nevertheless involve the ideas and utilities which, from the aspect from the prior art, are characteristic of the spirit of this invention and which, therefore, should and accordingly are intended to fall within the contemplation of the following claims. I, therefore, desire that all matter in the foregoing disclosure shall be interpreted as purely illustrative and not in a limiting sense, as it will be clear that the various steps and operations herein described may be identified by the use of various more or less arbitrary terms and that the terminology employed is descriptive rather than limiting.

Having thus amply disclosed my invention, what I claim as new and desire to secure by Letters Patent of the United States is:

1. A process of the nature disclosed for treating ores containing among other metallic constituents silver and large amounts of arsenic, consisting in subjecting the comminuted ore in a closed vessel to the action of moist chlorin gas at an elevated temperature, collecting the evolved vapors of arsenic chlorid and thus obtaining a residue free from arsenic, and then treating said residue to effect a separation of its valuable constituents.

2. A process of the nature disclosed for treating ores containing among other metallic constituents silver, nickel and arsenic, consisting in subjecting the comminuted ore to the action of moist chlorin gas at an elevated temperature, withdrawing the evolved arsenic chlorid from said vessel until the arsenic has been substantially removed from the residue, then leaching said residue, treating the insoluble matter to separate the silver therefrom, and treating the solution to separate the nickel therefrom.

3. A process of the nature disclosed for treating ores containing among other metallic constituents nickel, cobalt and arsenic, consisting in subjecting said ores in comminuted form to the action of moist chlorin gas for a period sufficient to convert substantially all the arsenic to arsenic chlorid, separating the vapors of arsenic chlorid from the residue, and then treating said residue

to effect an isolation of the nickel and the cobalt contained therein.

4. A process of the nature disclosed for treating ores containing silver, nickel, cobalt and arsenic, consisting in subjecting the comminuted ore to the action of moist chlorin gas for a time sufficient to convert substantially all of the arsenic to arsenic chlorid, separating the gaseous arsenic chlorid from the residue, leaching said residue to bring the nickel and cobalt compounds into solution, treating said solution to separate the nickel from the cobalt, and treating the insoluble silver-containing residue to separate the silver therefrom.

5. A process of the nature disclosed for treating ores containing among other metallic constituents nickel and considerable amounts of arsenic, consisting in subjecting the comminuted ore in a closed vessel to the action of moist chlorin gas at an elevated temperature, withdrawing the evolved vapors of arsenic chlorid and thus obtaining a residue free from arsenic, then leaching said residue to obtain a solution containing a compound of nickel, and then treating said solution to obtain metallic nickel therefrom.

6. A process of the nature disclosed for treating ores containing among other metallic constituents nickel and considerable amounts of arsenic, consisting in subjecting the comminuted ore in a closed vessel to the action of moist chlorin gas at a temperature of approximately 350° C., extracting excess quantities of heat engendered by said exothermic reaction to maintain the temperature as aforesaid, withdrawing the evolved vapors of arsenic chlorid, and then treating the residue to separate the nickel therefrom.

7. A process of the nature disclosed for treating ores containing among other metallic constituents silver and large amounts of arsenic, consisting in subjecting the comminuted ore in a closed vessel to the action of moist chlorin gas at an elevated temperature, extracting excess heat engendered by said exothermic action to maintain the temperature at approximately 350° C., withdrawing the evolved vapors of arsenic chlorid and thus obtaining a residue free from arsenic, and then treating said residue to effect a separation of its valuable constituents.

8. A process of the nature disclosed for treating ores containing among other metallic constituents silver, nickel, and arsenic, consisting in subjecting the comminuted ore to the action of moist chlorin gas at an elevated temperature, extracting the excess heat engendered by said exothermic reaction to maintain the temperature at approximately 350° C., withdrawing the evolved arsenic chlorid from said vessel until the arsenic has been substantially removed from

the residue, then leaching said residue, treating the insoluble matter to separate the silver therefrom, and treating the solution to separate the nickel therefrom.

5 9. A process of the nature disclosed for treating ores containing among other metallic constituents nickel, cobalt, and arsenic, consisting in subjecting said ores in comminuted form to the action of moist chlorin gas at an elevated temperature, extracting the excess heat engendered by said exothermic reaction to maintain the temperature at approximately 350° C., separating the vapors of arsenic chlorid from the residue, and then 10 treating said residue to effect an isolation of the nickel and cobalt contained therein.

10 10. A process of the nature disclosed for treating ores containing silver, nickel, cobalt and arsenic, consisting in subjecting 20 the comminuted ore to the action of moist chlorin gas at an elevated temperature, extracting excess heat engendered by said exothermic reaction to maintain the temperature at approximately 350° C., separating 25 the gaseous arsenic chlorid from the residue, leaching said residue to bring the nickel and cobalt compound to solution, treating said solution to separate the nickel from the cobalt, and treating the insoluble silver containing residue to separate the silver therefrom.

11 11. A process of the nature disclosed for treating ores containing among other metallic constituents nickel and large amounts 35 of arsenic, consisting in subjecting the comminuted ore in a closed vessel to the action of moist chlorin gas at an elevated temperature, maintaining a pressure less than atmospheric of gas within said closed vessel 40 to prevent any uncontrollable escape of vapors of arsenic chlorid, withdrawing the evolved vapors of arsenic chlorid and thus obtaining a residue free from arsenic, and then treating said residue to obtain the 45 nickel therefrom.

12 12. A process of the nature disclosed for treating ores containing among other metallic constituents silver and large amounts of arsenic, consisting in subjecting the comminuted ore in a closed vessel to the action 50 of moist chlorin gas at an elevated temperature, maintaining the gases within said vessel at a pressure less than atmospheric to prevent the uncontrollable escape of vapors 55 of arsenic chlorid, withdrawing the evolved vapors of arsenic chlorid from said vessel and thus obtaining a residue free from arsenic, and then treating said arsenic to obtain a separation of its valuable constituents.

60 13. A process of the nature disclosed for treating ores containing among other metallic constituents silver, nickel, and arsenic,

consisting in subjecting the comminuted ore to the action of moist chlorin gas at an elevated temperature, maintaining a pressure 65 less than atmospheric in the vessel containing said ore to prevent any uncontrollable escape of gases therefrom, withdrawing the evolved arsenic chlorid from said vessel until the arsenic has been substantially removed from the residue, then leaching said residue, treating the insoluble matter to separate the silver therefrom, and treating the solution to separate the nickel therefrom.

75 14. A process of the nature disclosed for treating ores containing among other metallic constituents nickel, cobalt and arsenic, consisting in subjecting said ores in comminuted form to the action of moist chlorin 80 gas for a period sufficient to convert substantially all the arsenic to arsenic chlorid, maintaining a pressure less than atmospheric in the vessel containing said ores to prevent any uncontrollable escape of gases, 85 withdrawing the gaseous arsenic chlorid from the residue, and then treating said residue to effect an isolation of the nickel and cobalt contained therein.

15. A process of the nature disclosed for 90 treating ores containing silver, nickel, cobalt and arsenic, consisting in subjecting the comminuted ore to the action of moist chlorin gas for a time sufficient to convert substantially all of the arsenic to arsenic chlorid, 95 maintaining a pressure less than atmospheric within the vessel containing said ores to prevent any uncontrollable escape of gases therefrom, withdrawing the gaseous arsenic chlorid from the residue, leaching 100 said residue to bring the nickel and cobalt compound into solution, treating said solution to separate the nickel from the cobalt, and treating the insoluble silver-containing residue to separate the nickel therefrom.

105 16. A process of the nature disclosed for treating ores containing among other metallic constituents silver and large amounts of arsenic, consisting in subjecting the comminuted ore at an elevated temperature and 110 in a state precluding granular agglomeration to the action of moist chlorin gas, withdrawing the evolved vapors of arsenic chlorid and thus obtaining a residue free from arsenic, and then treating said residue to 115 effect a separation of its valuable constituents.

In testimony whereof I affix my signature, in the presence of two witnesses.

WOOLSEY McA. JOHNSON.

Witnesses:

CHARLES M. STARKWEATHER,  
HARRY H. HOWARD.